

(Model.)

W. C. WALTER.

WALL PAPER.

No. 268,964.

Patented Dec. 12, 1882.

Fig. 1.



Fig. 2.



WITNESSES:

Carl Karp  
Otto Risch

INVENTOR

W. Charles Walter  
BY Paul Goepel

ATTORNEY

# UNITED STATES PATENT OFFICE.

W. CHARLES WALTER, OF NEW YORK, N. Y.

## WALL-PAPER.

SPECIFICATION forming part of Letters Patent No. 268,964, dated December 12, 1882.

Application filed January 24, 1881. (Model.)

To all whom it may concern:

Be it known that I, W. CHARLES WALTER, of the city, county, and State of New York, have invented certain new and useful Improvements in Wall-Papers, of which the following is a specification.

The object of this invention is to furnish an improved kind of wall-paper, to which a rich and plastic effect is imparted by coating and 10 decorating the surface with raised ornaments.

Heretofore a kind of plastic ornamentation of wall-papers has been obtained by employing flock, which, however, is expensive, as it 15 consists of short fibers of wool, and is mostly imported. My invention is designed to substitute therefor cheaper materials, and to produce a more variegated effect than with flock.

The invention consists of a wall-paper coated or decorated with properly-colored sand, sawdust, and ground glass, which are uniformly 20 distributed over the portions to be ornamented.

In the accompanying drawings, Figure 1 represents a top view of my improved wall-paper; and Fig. 2, a vertical transverse section of the same on line  $\alpha\alpha$ , Fig. 1.

Similar letters of reference indicate corresponding parts.

P represents paper or any other fabric, and A B C the raised ornamental portions, which 30 consist of properly-prepared sand, sawdust, and ground glass. The coating of the paper is accomplished in the customary manner by first laying on a coating of varnish, then distributing thereon the sand, sawdust, and ground 35 glass. The sand and sawdust are mixed with common sized colors and applied in dry state. The ground glass is coated with shellac-varnish and a bronze or other color, and then dis-

tributed over the varnished portions. The sawdust is screened after having been colored, 40 so that only the finest parts are used, it being designed as a substitute for the flock. The colored sand imparts an embroidery-like character to the ornaments produced, especially when laid upon a ground of colored glass. By 45 the ground glass a bronze-like or metallic coating is obtained, which is less expensive than bronze colors alone. A wall-paper of rich and characteristic appearance is finally obtained, which combines the effects of one or more of 50 the substances employed.

Having thus described my invention, I claim as new and desire to secure by Letters Patent—

1. As an article of manufacture, wall-paper 55 ornamented by surface coating or coating in figures of ground glass, sand, and sawdust previously prepared as herein described, and applied in a dry state to the face of the paper previously coated with varnish. 60

2. The method herein described of ornamenting wall-paper, consisting of the application of ground glass or glass pulverized, sand, and sawdust, prepared and colored as herein described, and applied in a dry state to the face of the 65 paper previously coated with varnish, as and for the purpose described.

In testimony that I claim the foregoing as my invention I have signed my name, in presence of two witnesses, this 13th day of January, 1881. 70

W. CHARLES WALTER.

Witnesses:

PAUL GOEPEL,  
CARL KARP.